# EUROPEAN PATENT SPECIFICATION

(11) **EP 2 661 400 B1**
(45) Date of publication and mention of the grant of the patent: **14.08.2019**
(21) Application number: 12701033.8
(22) Date of filing: 05.01.2012
(51) Int. Cl.: B65D 47/08

(54) **WET FRICTION MATERIAL FOR CLOSURES FOR PRODUCT CONTAINERS**
NASSREIBUNGSMATERIAL FÜR VERSCHLÜSSE VON PRODUKTAUFNAHMEBEHÄLTERN
MATÉRIAU À COEFFICIENT DE FROTTEMENT À L'ÉTAT HUMIDE ET DESTINÉ À DES FERMETURES POUR CONTENANTS DE PRODUIT

(30) Priority: 05.01.2011 US 201161429813 P; 20.12.2011 US 201113331353
(43) Date of publication of application: 13.11.2013
(73) Proprietor: The Gillette Company LLC, Boston, MA 02127 (US)
(72) Inventor: QUIGLEY, Steven, Francis, Kennebunkport, ME 04046 (US); GAJRIA, Chandrasen, Hingham, MA 02043 (US)
(74) Representative: Töpert, Verena Clarita
(86) International application number: PCT/US2012/020254
(87) International publication number: WO 2012/094442

(56) References cited:
- WO-A1-2009/071298
- WO-A2-2006/076747
- US-A- 2 394 135
- US-A- 3 972 528
- US-A- 5 443 172
- US-A1- 2007 020 025

## Description

### FIELD OF THE INVENTION

The invention generally relates to materials for closures for product containers, more particularly to materials for closures for product containers that have a high coefficient of friction when wet and low tack when dry.

### BACKGROUND OF THE INVENTION

Closures for product containers are intended to be grasped or handled by users. Such closures are typically made from a hard plastic such as thermoplastic polymers, e.g., polyethylene, polypropylene, and acrylonitrile butadiene styrene. These materials are inherently slippery, which results in slippage and/or poor engagement of the closure with a skin surface of a user. Moreover, such closures often have a small thickness when molded, which also may result in slippage and/or poor engagement of the closure with a skin surface of a user.

In addition, certain closures for product containers are typically used in wet or aqueous environments. For example, shampoo bottles are often used in the shower, which may further contribute to slippage and/or poor engagement of the bottle. Various product containers may hold lubricious materials, such as liquids, gels, non-aerosols, and foams that may spill onto the closure of the container, contributing to slippage and/or poor engagement of the container generally as well as in wet or aqueous environments.

Current approaches may increase the coefficient of friction when wet for a material, but these approaches, however, do not improve a user's perception of gripping or engaging thermoplastic polymers. In one approach, the thermoplastic polymer can have a higher coefficient of friction, but such approaches may also have higher tack or perception of stickiness to a user when dry, which may be uncomfortable and undesirable. In addition, current approaches have issues manufacturing materials that adhere to product containers.

What is needed, then, is a wet friction material suitable for a closure for a product container that preferably is stable and durable, and has a high coefficient of friction when wet and low tack when dry, which would improve engagement of the closure with a user's skin, e.g., for secure grip, potentially without discomfort. What is also needed is a wet friction material that can preferably adhere to or be formed with a product container.

US5443172 discusses a non-slip closure grip for a receptacle having an upper portion with external threads.

US3972528 discusses a friction grip for the handles of bats, rackets and the like which has a permanent tacky feel.

US2394135 discusses a closure for a container with inserts of plastic friction material.

US2007020025 discusses a combination container and applicator cap with an overshell providing a gripping surface on the cap.

WO06076747 discusses a screw top closure for a two liter bottle, with a resilient ring to provide purchase according to the preamble of claim 1.

WO09071298 discusses a cap for a container, the cap comprising a lid and an elastomeric pad.

### SUMMARY OF THE INVENTION

The invention provides a product container in accordance with the clams.

The one or more projections may be, for example, generally cylindrical projections, generally rectangular projections, generally knurled projections, ridges, non-linear ridges, and combinations thereof. The thermoplastic elastomer may define one or more pores to facilitate removal of water. The thermoplastic elastomer can have a coefficient of friction of in a range of about 2.0 to about 3.5 when wet with water, a tack force of about 3 g to about 12 g when dry, and/or a Shore A hardness of about 35 to about 50. The one or more projections can comprise at least two projections, and/or at least one groove can be formed between the at least two projections. The one or more projections can be integrally formed with the thermoplastic elastomer, for example, by injection molding. The closure further comprises a thermoplastic polymer. A coefficient of friction of the thermoplastic elastomer when wet is higher than a coefficient of friction of the thermoplastic polymer when wet. The thermoplastic elastomer can be formed with the thermoplastic polymer via injection molding, 2-step injection molding, 3-step injection molding, overmolding, and/or coextruding. The thermoplastic polymer can comprise polyethylene, polypropylene, acrylonitrile butadiene styrene, and combinations thereof.

### BRIEF DESCRIPTION OF THE DRAWINGS

Other features and advantages of the present invention, as well as the invention itself, can be more fully understood from the following description of the various embodiments, when read together with the accompanying drawings, in which:
FIG. 1 is a schematic front view of a product container;
FIG. 2 is a schematic perspective view of a known closure when wet;
FIG. 3 is a schematic perspective view of a wet friction material when wet, in accordance with an embodiment of the invention;
FIG. 4 is a chart illustrating the coefficient of friction of a wet friction material according to an embodiment of the invention when wet;
FIG. 5 is a chart illustrating properties of tack and coefficient of friction when wet for a wet friction material according to an embodiment of the invention;
FIG. 6 is a schematic perspective view of a textured surface in accordance with an embodiment of the invention;
FIG. 7 is a schematic perspective view of another textured surface in accordance with an embodiment of the invention;
FIG. 8 is a schematic perspective view of yet another textured surface in accordance with an embodiment of the invention; and
FIG. 9 is a schematic perspective view of still another textured surface according to an embodiment of the invention.

### DETAILED DESCRIPTION OF THE INVENTION

Except as otherwise noted, the articles "a," "an," and "the" mean "one or more."

Consumer goods, such as laundry and household cleaning products, shampoo and hair care products, oral care products, skin care products, and other personal care products that are typically used in wet environments or contain liquids or lubricious materials, are often packaged in various forms of articles, such as product containers. Closures (e.g., caps), such as hard plastics, on the product containers are often intended to prevent unintended release of the contents within the product containers and allow a user to dispense the contents. These closures are required to have a certain level of mechanical performance to prevent damage during transport and use, and also provide a level of aesthetic appeal to consumers. Nonlimiting examples of closures for product containers are described in U.S. Patent Nos. 3,661,300; 4,688,696; 6,013,270; and 6,036,036; U.S. Patent Application Publication Nos. 2007/0158230 and 2008/0245889; and PCT Publication Nos. WO 97/23387; WO 01/21499; WO 01/55002; WO 2007/049239; and WO 2010/088652.

Containers and closures manufactured from thermoplastic polymers, including polyolefins, polyethylene, acrylonitrile butadiene styrene (ABS), and polypropylene, can be manufactured in an extrusion blow molding process, an injection stretch blow process, and/or an injection molding process. Nonlimiting examples of thermoplastic polymers and processing thermoplastic polymers are described in U.S. Patent Nos. 4,619,803, 5,711,061, and 7,098,292 and U.S. Patent Application Publication Nos. 2005/0032969, 2006/0175738, 2007/0048473, 2008/0063824, and 2008/0150198. Suitable commercial grade thermoplastic polymers include polyethylene, such as high-density polyethylene or polyethylene terephtalate, and polypropylene are available from suppliers such as Borealis AG (Vienna, Austria), BP p.l.c. (London, United Kingdom), and Total Petrochemicals USA, Inc. (Houston, Texas), e.g., Total's PPR 7225.

Referring to FIGS. 1 and 2, a product container 10 comprises a housing 20 defining a hollow interior and a closure 30. The closure 30 is coupled to the housing 20 such that the closure covers, either directly or indirectly, the hollow interior. For example, the closure 30 can be coupled to the housing 20 via a screw-type arrangement, snap-fit connection, friction-fit connection, lock-and-key connection, male-female engagement, etc. Moreover, the closure 30 can comprise a first mounting member that corresponds in shape and mates with a second mounting member of the housing 20 to secure the closure 30 to the housing 20. The closure 30 can comprise a projection that mates with a recess of the housing 20 and/or the closure 30 can comprise a recess that mates with a projection of the housing 20. The projection of the closure 30 and/or the housing 20 can be rotationally asymmetric such that the coupling is accomplished in only a single orientation for securement. A portion 40 of the closure may have low surface energy and/or hydrophobic properties such that water on the portion 40 beads up when the closure 30 is wet with water.

The housing 20 of the product container 10 can hold a substance to be dispensed through the closure 30 or to prevent inadvertent release through the closure 30. In this regard, the housing 20 of the product container 10 can be a hard plastic, such as polyethylene, propylene, and ABS, phenolic, or a soft plastic, such as rubber, that can contain fluids or substances. For example, the product container 10 can contain soaps, detergents, toothpaste, shave preparations, gels, foams, aerosols, lotions, hair products, water, liquids, lubricious materials, cleaners, etc. In an embodiment in which the housing 20 of the product container 10 is formed from soft plastic, the housing 20 can be deformable to assist in dispensing the contents within the housing 20.

Referring now to FIG. 3, a wet friction material 50, a soft polymer, is disposed at least partially (or entirely) on the portion 40 of the closure 30. Additionally or alternatively, the wet friction material is disposed on, formed on, and/or formed with the portion 40 of the closure 30. The wet friction material 50 can be included on or with any skin-engaging portion of the closure 30. Additionally or alternatively, the wet friction material 50 is integrally formed or overmolded with the closure 30, e.g., in a two-stage or 3-stage molded process, an overmolding process, and/or a co-extrusion process. Nonlimiting examples of processing a soft polymer with a hard polymer (such as a hard plastic) are described in U.S. Patent No. 7,435,776; U.S. Patent Application Nos. 2009/0197107 and 2010/0152678; and "Novel Thermoplastic Elastomers for Universal Overmolding on Dissimilar Thermoplastics," by Liang Xu et al., available at www.glstpes.com/pdf/papers/2007%20topcon.pdf.

The wet friction material 50 has a high coefficient of friction when wet, e.g., higher coefficient of friction when wet compared to known thermoplastic polymers for product containers. The coefficient of friction is high for the wet friction material 50 when wet in aqueous environments, including water and lubricious materials (e.g., foams, gels, soaps, etc.), thus, facilitating improved engagement with the closure such that a user can more securely operate the closure in aqueous environments, including when the closure is at least partially covered with the contents within the product container 10. Furthermore, the wet friction material 50 may have a higher surface compliance than that of the known thermoplastic polymer for product containers, but preferably with low tack. For example, users can securely grip the wet friction material 50, e.g., resulting in improved comfort and control, when wet and not be uncomfortably grippy or sticky when dry. The wet friction material 50 is polar and hydrophilic. Additionally the wet friction material 50 has high surface energy (e.g., perhaps via a sufficiently low contact angle) so that wettability of the wet friction material 50 is improved and so that water beads are minimized or non-existent when the wet friction material 50 is wet with water. Without intending to be bound by any theory, it is believed that preventing water (or other lubricious materials) from beading and improving wettability (e.g., promoting surfacing wetting) may each or both serve to thin the amount of water that a user must penetrate to engage the skin to the wet friction material 50.

The wet friction material 50 comprises a thermoplastic elastomer. Nonlimiting examples of suitable thermoplastic elastomers are described in U.S. Patent Nos. 5,314,940, 5,670,263, 6,610,382, and 6,904,615; and U.S. Patent Application Publication Nos. 2002/0114920 and 2011/0143112. For example, suitable classes of elastomers may comprise hydrated styrene block copolymers (e.g., styrene-ethylene-butylene (SEBS) and styrene-butadiene-styrene (SBS)), anionic triblock copolymers, polyolefin-based thermoplastic elastomers, thermoplastic elastomers based on halogen-containing polyolefins, thermoplastic elastomers based on dynamically vulcanized elastomer-thermoplastic blends, thermoplastic polyether ester or polyester based elastomers, thermoplastic elastomers based on polyamides or polyimides, ionomeric thermoplastic elastomers, partially or fully hydrogenated styrene-butadiene-styrene block copolymers, hydrogenated block copolymers in thermoplastic elastomer interpenetrating polymer networks, thermoplastic elastomers by carbocationic polymerization, polymer blends containing styrene/ hydrogenated butadiene block copolymers, block polymers such as polystyrene materials with elastomeric segments, and polyacrylate-based thermoplastic elastomers. Examples of elastomers may include natural rubber, butyl rubber, EPDM rubber, silicone rubber such as polydimethyl siloxane, polyisoprene, polypropylene, polybutadiene, polyurethane, ethylene/propylene/diene terpolymer elastomers, chloroprene rubber, styrene-butadiene copolymers (random or block), styrene-isoprene copolymers (random or block), acrylonitrile-butadiene copolymers, mixtures thereof and copolymers thereof. The block copolymers may be linear, radial or star configurations and may be diblock (AB) or triblock (ABA) copolymers or mixtures thereof. Blends or combinations of these elastomers with each other or with modifying non-elastomers are also contemplated. Elastomers may be available from Arkema Inc., Philadelphia, Pennsylvania (e.g., Pebax® 2533); E. I. duPont de Nemours & Co., Wilmington, Delaware (e.g., Zytel® 158L); Kraiburg TPE Corp., Duluth, Georgia; and Kraton Polymers U.S. LLC, Houston, Texas.

Additionally or alternatively, the wet friction material 50 is a composite structure, such as a thermoplastic elastomer modified with additives, fillers, and/or rubber mixtures or modifiers. Suitable composite structures, additives, and/or fillers are described in U.S. Patent No. 3,972,528. For examples, additives may be one or more of the following additives: paraffinic white oils, inorganic bulking agents, ether ester plasticizers, sulfurized mineral oil, alkenyl amide, styrol, polystyrol, petrolatum, polyisobutylene, polybutene, styrene, elastomeric styrene, ethylene, butylene, aqueous carboxylated synthetic polymer having a minimum film-forming temperature (MFFT) (e.g., 10 degrees Celsius or below), low MFFT synthetic polymer reinforced during manufacturing by co-agglomeration with polystyrene, combinations thereof, or any other suitable additive to achieve a wet friction material 50 that has a high coefficient of friction when wet and low tack when dry. Additionally or alternatively, fillers may be one or more if the following fillers: clay treated with lignin sulfonate, pulverized fragments of foamed melamine resin, porous granulated aluminum oxide powder, diatomaceous earth, silica, acrylonitrile pulp, granular filler having a surface area of about 35 m²/g to about 410 m²/g, clay (about 5 parts by weight to about 30 parts by weight), aluminum hydroxide, hollow aluminum oxide particle, dibutylphtalate (applied on carbon fiber base material) that has been hardened, fired, and carbonized), vulcanized rubber particles, aramid fiber, waste ash, ethylene vinyl acetate, polyethelyene, rubber, elastomer, hollow carbonate, alumina, carbide, carborundum, diamond powder, white carbon (about 15 percentage by weight to about 80 percentage by weight), ceramic fiber (about 5 percentage by weight to about 50 percentage by weight), combinations thereof, or any other suitable filler to achieve a wet friction material 50 that has a high coefficient of friction when wet and low tack when dry. The quantity of any additives and/or fillers is controlled such that tensile strength is maintained at an acceptable level with adhesion to a substrate also being maintained at an acceptable level.

FIGS. 4 and 5 illustrate various properties, such as coefficient of friction when wet and tack force when dry, wet friction materials A and B. Tack is a characteristic of a material to form an immediate cohesive adherence to a contacting surface. Therefore, tack form is the measure of resistance of the material to separate from the contacting surface. In an embodiment, wet friction material A has a coefficient of friction when wet with water of about 2.8. The tack force of the wet friction material B can be similar to that of the known thermoplastic polymer for the closure 30, though the tack force of wet friction materials can be greater than or lesser than the known thermoplastic polymer for the closure 30. The tack force of the wet friction material B is in a range of about 1 g to about 25 g, preferably about 3 g to about 12 g. In alternative embodiments, the tack force of a wet friction material in accordance with an embodiment of the invention can be much higher than that of the known thermoplastic polymer for the closure 30. For example, the tack force of a wet friction material can be in a range of about 200 g to about 700 g, preferably about 300 g to about 500 g. The coefficient of friction when wet with water for the wet friction material B is preferably in a range of about 2.1 to about 3.2, and even more preferably about 2.4 to about 2.8. The coefficient of friction when wet with lubricious material, for example, using about 2 g of Gillette® Series Sensitive Skin Shave Gel, wet friction materials according to embodiments of the invention is preferably in a range of about 0.28 to about 2.0, and even more preferably about 0.29 to about 0.5.

Generally, wet friction materials of the invention have a higher coefficient of friction when dry, higher coefficient of friction when wet, higher surface energy, higher peel strength, which relate to strength of an adhesive bond, e.g., to a substrate, than known thermoplastic polymers for closures. Additionally or alternatively, the hardness of a wet friction material can be in a range of Shore A hardness of about 5 to about 95, preferably about 30 to about 60, and even more preferably about 35 to about 53. The coefficient of friction when dry for wet friction materials can be in a range of about 2.0 to about 5.3, preferably about 2.4 to about 3.0. The coefficient of friction when wet with water for wet friction materials can be in a range of about 1.4 to about 5.0, preferably about 1.9 to about 2.8. Surface energies of wet friction materials can be in a range of about 25 mJ/m² to about 52 mJ/m², preferably about 27 mJ/m² to about 34 mJ/m².

Referring now to FIGS. 6 through 9, various embodiments of wet friction materials of the present invention can optionally include projections or textured patterns extending from the wet friction material to improve engagement of the wet friction material with a skin. The projections and textured patterns can also break the surface tension of the water (or lubricious material) or be exposed above the water (or lubricious material) for engagement with skin. In one embodiment, a textured pattern 60 can be similar to that of a fingerprint pattern with nonlinear shapes, concave and/or convex curvatures, and intersecting lines. In another embodiment, projections 70 can have a generally rectangular shape, such that a cross-section of each of the projections 70 is generally square. By "generally rectangular" the projections 70 include non-rectangular elements, e.g., ridges, protrusions, or recesses, and/or may include regions along its length that are not rectangular, such as tapered and/or flared ends due to manufacturing and design considerations. In yet another embodiment, projections 80 can be generally cylindrical, such that a cross section of the each of the projections 80 can be generally circular. By "generally cylindrical" the projections 80 include non-cylindrical elements, e.g., ridges, protrusions, or recesses, and/or may include regions along its length that are not cylindrical, such as tapered and/or flared ends due to manufacturing and design considerations. In still another embodiment, projections 90 can be generally knurled, such that a cross-section of each of the projections 90 can be generally diamond-shaped. The projections can form any geometric, polygonal, arcuate shape, or combinations thereof. For example, the projections can include a combination of a knurled pattern and arcuate ridges. In an embodiment, the projections and/or the textured patterns are integrally formed with the wet friction material. Additionally or alternatively, the projections and/or textured patterns can be configured and shaped to form channels for fluid removal. The channels can be grooves formed between the projections. In an additional or alternative embodiment, the channels can define pores to remove/wick fluid away from the wet friction material by absorbing fluids, e.g., via an absorbent layer beneath the wet friction material, or by allowing the fluid to drain underneath the wet friction material. In various embodiments, without intending to be bound by any theory, it is believed that a range of percentage ratios of the distance between projections (D) over the height of the projections (H) promote pleasant sensory touch, preferably in a range of about 25% to about 75%, even more preferably about 60%. Further, it is believed that the less feedback of the projection on the skin surface, such as a fingertip, provides a more comfortable feeling. For example, the less feedback of the projection, that is a larger surface area to touch the skin, is more comfortable; in contrast, the higher feedback of the projection, that is a smaller surface area or a shaper edge, to touch a skin is less comfortable.

### TEST PROCEDURE FOR MEASURING PROPERTIES

### HARDNESS

Hardness of materials is tested at room temperature and at 36 degrees Celsius using Shore A Durometer Instron Model 9130-35 (available from Instron, Norwood, Massachusetts) according to ASTM 2240-00.

### COEFFICIENT OF FRICTION WHEN DRY AND WHEN WET

Coefficient of friction for each material to be tested is measured using a MTT175 tensile tester (available from Dia-stron Limited, Broomall, Pennsylvania) in which a skin mimic preparation is dragged across the material to be tested. The coefficient of friction for each material is tested when dry, wet with water, or in the presence of various lubricious materials (e.g., foams, gels, non-aerosols). To mimic skin, a polyurethane textured pad is prepared. Nonlimiting examples of skin mimic preparations and polyurethane textured pads are described in U.S. Patent Application Publication Nos. 2007/0128255 and 2009/0212454. A sled/probe is used in which the surface is polished stainless steel. The skin mimic is attached to the sled/probe surface via double-sided tape or clips. The material to be tested is attached to the stage below the sled/probe surface with preferably double-sided tape and optionally clips. If heat is used, the water bath to warm the platform of the MTT175 tester is set to 39 +/- 1 degrees Celsius and water is circulated. The sled/probe with the skin mimic is mounted to the floating parallelogram cradle of the tester, which is connected to a load cell. The angle of the sled/probe with the skin mimic is set so that the skin mimic surface is flat against the stage, which is attached to the material to be tested, with an approximate angle of about 35 degrees. The parallelogram cradle is leveled to be flat. Downward force can be adjusted by moving weights along a threaded shaft in which the downward force is adjusted to about 175 gm to about 230 gm. If shave preparations (e.g., lubricious materials) are used, lather is generated by applying the shave preparation to the material to be tested, lathering by hand for about 30 seconds to about 60 seconds. For gels, 2.5 +/- 0.7 grams of gel is applied. For foams, 3.0 +/- 0.7 grams of foam is applied. A draw down bar can be used to level the surface of the shave preparation, set at about 2 mm, across the skin mimic. Before performing the tests, the load cells are zeroed. To run the test measuring the coefficient of friction, software associated with the MTT175 tester is used and set at about 2000 gmf load cell with a displacement of about 60 mm and a speed of about 1500 mm/min at room temperature. Of the displacement, a smaller range of displacement is analyzed, such as about 110 mm to about 150 mm. A force of about 226 g is applied in which the force is calibrated with a Mettler-Toldeo Balance Serial No. 114020837 (available from Mettler-Toledo, Inc., Columbus, Ohio). When measuring the coefficient of friction when wet, about 1 mL of room temperature tap water under the probe is used. About one to about three strokes are completed for each test and about three tests completed for each material. To perform another test, a new material is used. The skin mimic on the test head is washed with water and an alcohol wipe, then blotted dry with a paper towel. Alternatively, the skin mimic is replaced. The test head is dried before use.

To maximize reliability of data, at least three different operators perform the tests with a relative standard deviation of about less than 20% for the first stroke data over three separate tests - each operator over a period of three separate days. For each operator, the relative standard deviation is about less than 20%.

### TACK

Tack information for each material is measured using a TA.XT*Plus* Texture Analyzer and its associated software (available from Texture Technologies Corporation, Scarsdale, New York). Skin mimic, as prepared as described above, is attached to the round probe end of the Texture Analyzer instrument via double-sided tape and the material to be tested is attached to the metal stage of the Texture Analyzer instrument, which is below the Tack probe, via double-sided tape. The instrument is calibrated such that the height is set at 10 mm and the force is set using a 2000 g weight. Each cycle of testing includes probe contact with the material to be tested for about 5 seconds. The probe contact is then pulled away at about 5 mm/second. The probe contacts the material to be tested a second time for about 5 seconds and is then pulled away at about 1 mm/second. Optionally, to maximize good, repeatable contact of the probe with the material to be tested, the probe contacts the material for the second time after about a 5 second delay.

After a cycle of testing is complete, the skin mimic is washed with alcohol and is blotted dry with a paper towel. The material to be tested is replaced with a fresh, new material and repeated for a total of at least three cycles of sampling per material.

To maximize reliability of data, at least three different operators perform the tests with a relative standard deviation of about less than 50%, preferably about less than 20%, over three separate tests - each operator over a period of three separate days.

### SURFACE ENERGY

Contact angle measurements is used to determine the surface energy of the materials to be tested in which the contact angle depends on the compatibility between the surface properties of the wetting liquid and the material to be tested. Surface energy is calculated from Young's equation in measures of energy per unit area (mJ/m²). Contact angle measurements utilize a Contact Angle and Surface Tension instrument (available from First Ten Angstroms, Portsmouth, Virginia), such as FTA200, with FTA video 2.0 software in which the instrument includes a camera that can capture many frames per second, a pump to dispense drops from syringes, and a stage to place the sample while frames are collected. To set up the test, the lighting is adjusted so that there is a white background and a dark drop and the focus is adjusted.

The material to be tested is placed below the syringe and leveled. The syringe is filled with a first liquid such that no bubbles remain. The program is initiated and run such that the instrument drops the liquid and takes measurements of contact angle. Two solvents are used, specifically diiodomethane and water. Owens-Wendt regression analysis is conducted to obtain surface energy measurements based on these two solvents.

It should be understood that every maximum numerical limitation given throughout this specification includes every lower numerical limitation, as if such lower numerical limitations were expressly written herein. Every minimum numerical limitation given throughout this specification includes every higher numerical limitation, as if such higher numerical limitations were expressly written herein. Every numerical range given throughout this specification includes every narrower numerical range that falls within such broader numerical range, as if such narrower numerical ranges were all expressly written herein.

All parts, ratios, and percentages herein, in the Specification, Examples, and Claims, are by weight and all numerical limits are used with the normal degree of accuracy afforded by the art, unless otherwise specified.

The dimensions and values disclosed herein are not to be understood as being strictly limited to the exact numerical values recited. Instead, unless otherwise specified, each such dimension is intended to mean both the recited value and a functionally equivalent range surrounding that value. For example, a dimension disclosed as "40 mm" is intended to mean "about 40 mm."

While particular embodiments of the present invention have been illustrated and described, it would be obvious to those skilled in the art that various other changes and modifications can be made without departing from the scope of the invention. It is therefore intended to cover in the appended claims all such changes and modifications that are within the scope of this invention.

## Claims

1. A product container (10) comprising:
a housing (20) defining a hollow interior; and
a closure (30)coupled to the housing (20) such that the closure (30) covers an opening to the hollow interior, wherein the closure (30) comprises a textured thermoplastic elastomer (50) on at least a portion (40) of the closure (30), wherein the thermoplastic elastomer comprises one or more projections extending therefrom, **characterized in that** the thermoplastic elastomer (50) is hydrophilic and polar.

2. The product container of claim 1, wherein the thermoplastic elastomer defines one or more pores to facilitate removal of water.

3. The product container of claim 1 that has one or more of the following features:
(i) the one or more projections is selected from the group consisting of generally cylindrical projections, generally rectangular projections, generally knurled projections, ridges, non-linear ridges, and combinations thereof;
(ii) the one or more projections comprises at least two projections and at least one groove can be formed between the at least two projections.
(iii) the one or more projections is integrally formed with the thermoplastic elastomer and, optionally, the one or more projections is integrally formed with the thermoplastic elastomer by injection molding.

4. The product container of any of claims 1 to 3, wherein the closure further comprises a thermoplastic polymer.

5. The product container of claim 4 that has one or more of the following features:
(i) a coefficient of friction of the thermoplastic elastomer when wet is higher than a coefficient of friction of the thermoplastic polymer when wet;
(ii) the thermoplastic elastomer is formed with the thermoplastic polymer via injection molding, 2-step injection molding, 3-step injection molding, overmolding, and/or coextruding.
(iii) the thermoplastic polymer is selected from the group consisting of polyethylene, polypropylene, and combinations thereof.

## Patentansprüche

1. Produktbehälter (10), umfassend:
ein Gehäuse (20), das einen hohlen Innenraum definiert; und
einen Verschluss (30), der mit dem Gehäuse (20) derart verbunden ist, dass der Verschluss (30) eine Öffnung zum hohlen Innenraum abdeckt, wobei der Verschluss (30) ein strukturiertes Thermoplastelastomer (50) auf wenigstens einem Teil (40) des Verschlusses (30) umfasst, wobei das thermoplastische Elastomer einen oder mehrere Vorsprünge umfasst, die sich davon erstrecken, **dadurch gekennzeichnet, dass** das Thermoplastelastomer (50) hydrophil und polar ist.

2. Produktbehälter nach Anspruch 1, wobei das Thermoplastelastomer ein oder mehrere Poren definiert, um das Entfernen von Wasser zu erleichtern.

3. Produktbehälter nach Anspruch 1, das eines oder mehrere der folgenden Merkmale aufweist:
(i) die ein oder mehreren Vorsprünge sind ausgewählt aus der Gruppe bestehend aus im Allgemeinen zylindrischen Vorsprüngen, im Allgemeinen rechteckigen Vorsprüngen, im Allgemeinen geriffelten Vorsprüngen, Rippen, nicht-linearen Rippen und Kombinationen davon;
(ii) die ein oder mehreren Vorsprünge umfassen wenigstens zwei Vorsprünge und es kann wenigstens eine Rille zwischen den mindestens zwei Vorsprüngen ausgebildet sein.
(iii) die ein oder mehreren Vorsprünge sind integral mit dem Thermoplastelastomer geformt und die ein oder mehreren Vorsprünge sind wahlweise mit dem Thermoplastelastomer durch Spritzgießen geformt.

4. Produktbehälter nach einem der Ansprüche 1 bis 3, wobei der Verschluss ferner ein thermoplastisches Polymer umfasst.

5. Produktbehälter nach Anspruch 4, das eines oder mehrere der folgenden Merkmale aufweist:
(i) einen Reibungskoeffizienten des Thermoplastelastomers, der, wenn es nass ist, höher ist als ein Reibungskoeffizient des Thermoplastpolymers, wenn es nass ist;
(ii) das Thermoplastelastomer ist mit dem Thermoplastpolymer durch Spritzgießen, 2-stufiges Spritzgießen, 3-stufiges Spritzgießen, Umspritzen und/oder Coextrudieren geformt.
(iii) das Thermoplastpolymer ist ausgewählt aus der Gruppe bestehend aus Polyethylen, Polypropylen und Mischungen davon.

## Revendications

1. Contenant de produit (10) comprenant :
un logement (20) définissant un intérieur creux ; et
une fermeture (30) couplée au logement (20) de telle sorte que la fermeture (30) couvre une ouverture vers l'intérieur creux, dans laquelle la fermeture (30) comprend un élastomère thermoplastique texturé (50) sur au moins une partie (40) de la fermeture (30), dans laquelle l'élastomère thermoplastique comprend une ou plusieurs saillies s'étendant à partir de là, **caractérisé en ce que** l'élastomère thermoplastique (50) est hydrophile et polaire.

2. Contenant de produit selon la revendication 1, dans lequel l'élastomère thermoplastique définit un ou plusieurs pores pour faciliter l'élimination de l'eau.

3. Contenant de produit selon la revendication 1 qui possède une ou plusieurs des caractéristiques suivantes :
(i) les une ou plusieurs saillies sont choisies dans le groupe constitué de saillies généralement cylindriques, saillies généralement rectangulaires, saillies généralement moletées, crêtes, crêtes non linéaires, et leurs combinaisons ;
(ii) les une ou plusieurs saillies comprennent au moins deux saillies et au moins une rainure peut être formée entre les au moins deux saillies.
(iii) les une ou plusieurs saillies sont formées en une seule pièce avec l'élastomère thermoplastique et, facultativement, les une ou plusieurs saillies sont formées en une seule pièce avec l'élastomère thermoplastique par moulage par injection.

4. Contenant pour produit selon l'une quelconque des revendications 1 à 3, dans lequel la fermeture comprend en outre un polymère thermoplastique.

5. Contenant de produit selon la revendication 4 qui possède une ou plusieurs des caractéristiques suivantes :
(i) un coefficient de frottement de l'élastomère thermoplastique lorsqu'il est humide est supérieur à un coefficient de frottement du polymère thermoplastique lorsqu'il est humide ;
(ii) l'élastomère thermoplastique est formé avec le polymère thermoplastique par moulage par injection, moulage par injection en 2 étapes, moulage par injection en 3 étapes, surmoulage, et/ou coextrusion.
(iii) le polymère thermoplastique est choisi dans le groupe constitué de polyéthylène, polypropylène, et leurs combinaisons ;
